

July 14, 1925.

1,545,591

J. J. MADINE

MANUFACTURE OF ELECTRON DISCHARGE DEVICES

Filed March 6, 1923



Fig. 2



Fig. 3



Inventor:  
John J. Madine,  
by *Jel Ch. Palmer* ATT'y.

## UNITED STATES PATENT OFFICE.

JOHN J. MADINE, OF NEWARK, NEW JERSEY, ASSIGNOR TO WESTERN ELECTRIC COMPANY, INCORPORATED, OF NEW YORK, N. Y., A CORPORATION OF NEW YORK.

## MANUFACTURE OF ELECTRON-DISCHARGE DEVICES.

Application filed March 6, 1923. Serial No. 623,188.

To all whom it may concern:

Be it known that I, JOHN J. MADINE, a citizen of the United States, residing at Newark, in the county of Essex, State of New Jersey, have invented certain new and useful Improvements in the Manufacture of Electron-Discharge Devices, of which the following is a full, clear, concise, and exact description.

10 This invention relates to the manufacture of electron discharge devices such as vacuum tubes and has for its object a tight seal between the leading-in wires and the glass envelope.

15 The enclosing vessel of an electron discharge device consists of a tube or envelope ordinarily composed of lead glass to which is fused a stem composed of the more expensive potash glass. The reason for using 20 potash glass in the stem lies in the fact that platinum seals much better in potash glass than it does in lead glass. Lead glass is used to reduce the cost of the device as it is less expensive than potash glass but 25 equally good as an envelope.

In electron discharge devices having large potential differences impressed between the grid and anode it is not practical to seal all the leading-in wires in the press at the 30 end of the stem because the leading-in wires for the anode and grid cannot be placed sufficiently far apart to obtain the necessary insulation. It is therefore common practice in tubes of this character to seal in the 35 leading-in wires for the anode and grid at the juncture of the stem flare and the envelope at points opposite each other so that the necessary insulation is obtained.

40 This invention insures a tight seal for these leading-in wires by providing on the platinum portion of the leading-in wire a bead of potash glass which is fused to the glass of the containing vessel, the bead being fused to the vessel to close an aperture 45 formed therein after the stem and flare have been united to form the enclosing vessel for the device.

50 Referring now to the drawings Fig. 1 discloses the envelope and stem in position to be united together, the stem carrying the electrode assembly. Fig. 2 discloses a step in the process of sealing in the grid and anode leading-in wires, and Fig. 3 discloses the finished seal.

55 In Fig. 1, 10 is a lead glass envelope and

11 is the stem from which is supported the electrode assembly 12. The leading-in wires 13 for the cathode are sealed in the press at the end of the stem. The leading-in wire 14 for the grid electrode comprises a coil of 60 wire from the lower end of which is suspended a short piece of platinum wire 15. The leading-in wire 16 for the anode likewise comprises a coil of wire and a piece of platinum wire 17.

65 The sealing of the stem to the envelope and the sealing in of the platinum wires 15 and 17 is accomplished in the following manner:

The lower rim of the envelope 10 and the 70 rim of the flare of the stem 11 are softened by a flame and fused together in the ordinary manner with the lead wires 14 and 15 drawn up within the vessel due to the coils therein. After the stem and envelope have 75 been fused together small apertures, as shown at 18 in Fig. 2, are blown at the juncture of the stem and envelope rim in general alignment with the leading-in wires 14 and 16. Short glass tubes 19 are fused to the 80 glass vessel in alignment with the apertures. A tool is now thrust through each tube 19 and its corresponding aperture, and the end of a leading wire gripped and pulled out so that the platinum portion lies outside the 85 vessel. A bead 20 of potash glass is applied to the platinum portion and is then fused to the end of a tube 19 to close it, resulting in the arrangement shown in 90 Fig. 3.

95 This insures a tight seal for the leading-in wires as the bead of potash glass seals tightly to the platinum portion of the leading-in wires and then fuses to the tube 19 to form a gas-tight vessel. The use of the glass tubes 19 reduces the number of devices defective because of cracked seals. For, any crack developing around the seal during subsequent heating in evacuating the device is limited to the tubes and does not extend 100 to the vessel itself. It is, therefore, possible to merely soften the glass of the tubes 19 and by slight manipulation close such a crack with little effort, whereas if the crack had extended to the vessel itself much working would not be possible.

105 What is claimed is:

110 1. The method of manufacturing electron discharge devices which comprises fusing together an envelope and stem of different

- types of glass, forming an aperture at the juncture of said different types, arranging a leading-in wire in said aperture, applying a bead of glass to said leading-in wire, and fusing said bead to the remaining glass to close said aperture. 5
2. The method of manufacturing electron discharge devices which comprises mounting an electrode assembly upon a stem, sealing said stem to an envelope with certain of the leading-in wires completely within the vessel, forming holes in the vessel, drawing said leading-in wires through said holes, applying glass beads to said leading-in wires, and closing said holes with said beads. 10
3. In an electron discharge device, a vessel comprising an envelope of one type of glass, a stem of another type of glass, electrodes supported by said stem, leading-in wires for said electrodes passing through said vessel at the juncture of said envelope and said stem, and a bead of the same kind of glass as the stem surrounding said leading-in wire and fused to said containing vessel. 15
4. The method of manufacturing electron discharge devices which comprises forming an aperture in the enclosing vessel thereof, drawing a leading-in wire through said aperture, applying a bead of glass to said leading-in wire, and sealing said glass bead to said envelope to close said aperture. 20
5. The method of manufacturing electron discharge devices which comprises fusing together an envelope of lead glass and a stem of potash glass to form an enclosing vessel, forming an aperture at the juncture of said potash and lead glass, applying a bead of potash glass to a leading-in wire, and fusing said bead to the enclosing vessel to close said aperture. 40
6. In an electron discharge device, an enclosing vessel comprising an envelope of lead glass and a stem of potash glass, electrodes supported from said stem, leading-in wires for said electrodes passing through said vessel at the juncture of said envelope and said stem, and a bead of potash glass surrounding said leading-in wire and fused to said enclosing vessel. 45
7. In an electron discharge device, an enclosing vessel comprising an envelope and a stem, an electrode supported from said stem, a leading-in wire for said electrode passing through said vessel at the juncture of said envelope and stem, a glass tube sealed to said vessel and enclosing said leading wire, and a glass bead fused to said leading-in wire and to the end of said tube. 50
8. The method of manufacturing electron discharge devices which comprises fusing together an envelope and a stem of different kinds of glass to form a containing vessel, forming an aperture at the juncture of said stem and envelope, fusing a glass tube to said vessel in alignment with said aperture, fusing a bead of glass to a leading-in wire, and closing said tube with said bead. 55

In witness whereof, I hereunto subscribe my name this 1st day of March A. D., 1923.

JOHN J. MADINE.